

# UNITED STATES PATENT OFFICE.

HERBERT ABRAHAM, OF NEW YORK, N. Y.

## ROOFING MATERIAL.

1,226,738.

Specification of Letters Patent. Patented May 22, 1917.

No Drawing.

Application filed February 27, 1917. Serial No. 151,170.

To all whom it may concern:

Be it known that I, HERBERT ABRAHAM, a citizen of the United States, residing at the city, county, and State of New York, have invented certain new and useful Improvements in Roofing Materials, of which the following is a specification.

My invention relates to waterproof roofing materials of the kind known commonly as flexible prepared roofings, also prepared roofing shingles, which consist of a felted fabric either saturated, or saturated and coated, with bituminous materials. The invention applies more particularly to the felted fabric used in the manufacture of such roofings.

According to my invention I use certain varieties of marine plants of a fibrous nature, particularly sea grass or eel grass of the *Naiadaceae* family, for the production of the fibrous felt. Sea grass grows in both fresh and salt water, and can be readily and cheaply obtained in large quantities. It resists decay to a remarkable degree when exposed to the elements, and also withstands fire in that it does not readily ignite in its air-dry state.

I have found that felt containing sea grass has good tensile strength and porosity, and is much cheaper to manufacture than felt made from cotton and woolen rags, jute or other ligneous fibers or paper pulp.

In practising my invention, I first disintegrate the rag fibers in a beating machine in the usual manner. To the fibrillous mass or pulp consisting of the rag fibers suspended in water, I add a quantity of the sea grass in its raw or natural state, that is without being previously treated chemically.

I have obtained very satisfactory results by using a mixture containing approximately 25% of sea grass based on the dry weight. The sea grass fibers can either be added alone or with a suitable quantity of waste papers. The mixture is then beaten to bring it to a properly shredded condition.

The stock is then run into sheets of the desired size and thickness on a felt machine common to the felt and paper industries, and the sheets thus formed are dried.

This felt is subsequently either impregnated with tar to form the article of com-

merce known as "tarred felt," or else with asphalt to form what is known commercially as "asphalt saturated felt." The felt 55 may similarly be impregnated with a soft bituminous material and then surfaced with a bituminous material of a harder consistency to form what is known commercially as "flexible prepared roofing," or it 60 may be further treated with particles of crushed slate or other mineral material embedded on the surface and cut into smaller units to form what is known commercially as "prepared roofing shingles." 65

It has been customary to add waste papers (composed of either mechanically ground or chemically treated paper fibers) to the rag fibers, either to cheapen or else to suitably harden the latter. In practice, however, it has not been found possible to use more than about half paper fibers to half rag fibers based on their dry weight, without detracting from the porosity or pliability of the felt. I have found that the use of sea 75 grass fibers in conjunction with the paper fibers will overcome these tendencies, and will produce a sheet which on account of its porosity will saturate well with the bituminous material, and at the same time will 80 present greater pliability than if the paper stock alone were used. Thus for example I have obtained very good results by using a mixture composed of 25% of sea grass, 40% of paper stock, and 35% of rag stock 85 based on their dry weights, but it is not to be understood that I limit myself to these specific proportions, as even larger quantities of the sea grass can be used in case it is 90 so desired.

The felted fabric herein described is intended primarily for use in the manufacture of prepared roofings, including shingles, but it is not to be understood that I limit myself to that particular use of the 95 material, as it may be used for other purposes.

What I claim as my invention and desire to secure by Letters Patent is:

1. A prepared roofing comprising a felt 100 containing sea grass waterproofed with bituminous substances.

2. A prepared roofing comprising a felt composed of a mixture of rags and sea grass

fibers waterproofed with bituminous substances.

3. A prepared roofing comprising a felt composed of a mixture of rags, paper and 5 sea grass fibers waterproofed with bituminous substances.

4. A felted sheet formed of a beaten pulp containing a mixture of sea grass fibers

which have not been treated chemically, with rag fibers.

5. A felted sheet formed of a beaten pulp containing sea grass fibers which have not been treated chemically, with rag and paper fibers.

HERBERT ABRAHAM.